



US010144115B2

(12) **United States Patent**  
**Veneziale et al.**

(10) **Patent No.:** **US 10,144,115 B2**  
(45) **Date of Patent:** **\*Dec. 4, 2018**

(54) **METHOD OF MAKING POLISHING LAYER FOR CHEMICAL MECHANICAL POLISHING PAD**

(71) Applicants: **Rohm and Haas Electronic Materials CMP Holdings, Inc.**, Newark, DE (US); **Dow Global Technologies LLC**, Midland, MI (US)

(72) Inventors: **David Michael Veneziale**, Hatfield, PA (US); **Bainian Qian**, Newark, DE (US); **Teresa Brugarolas Brufau**, Philadelphia, PA (US); **Julia Kozhukh**, Bear, DE (US); **Yuhua Tong**, Hockessin, DE (US); **Jeffrey B. Miller**, West Chester, PA (US); **Diego Lugo**, Newark, DE (US); **George C. Jacob**, Newark, DE (US); **Marty W. DeGroot**, Middletown, DE (US); **Andrew Wank**, Avondale, PA (US); **Fengji Yeh**, Wilmington, DE (US)

(73) Assignees: **Rohm and Haas Electronic Materials CMP Holdings, Inc.**, Newark, DE (US); **Dow Global Technologies LLC**, Midland, MI (US)

(\*) Notice: Subject to any disclaimer, the term of this patent is extended or adjusted under 35 U.S.C. 154(b) by 102 days.

This patent is subject to a terminal disclaimer.

(21) Appl. No.: **15/163,213**

(22) Filed: **May 24, 2016**

(65) **Prior Publication Data**

US 2016/0375555 A1 Dec. 29, 2016

**Related U.S. Application Data**

(63) Continuation-in-part of application No. 14/751,423, filed on Jun. 26, 2015.

(51) **Int. Cl.**  
**B24D 18/00** (2006.01)  
**B24B 37/24** (2012.01)

(Continued)

(52) **U.S. Cl.**  
CPC ..... **B24D 18/0009** (2013.01); **B24B 37/24** (2013.01)

(58) **Field of Classification Search**  
CPC ..... B24D 18/00; B24B 37/24; H01L 21/302;  
H01L 21/00  
See application file for complete search history.

(56) **References Cited**

**U.S. PATENT DOCUMENTS**

3,677,681 A 7/1972 Zippel et al.  
3,705,821 A 12/1972 Breer et al.  
(Continued)

**FOREIGN PATENT DOCUMENTS**

JP 2001172732 12/2002

*Primary Examiner* — Pegah Parvini

(74) *Attorney, Agent, or Firm* — Andrew Merriam; Blake T. Biederman

(57) **ABSTRACT**

A method of forming a chemical mechanical polishing pad polishing layer is provided, including: providing a mold having a base with a negative of a groove pattern; providing a poly side (P) liquid component; providing an iso side (I) liquid component; providing a pressurized gas; providing an axial mixing device; introducing the poly side (P) liquid component, the iso side (I) liquid component and the pressurized gas to the axial mixing device to form a combination; discharging the combination from the axial mixing device at a velocity of 5 to 1,000 m/sec toward the base; allowing the combination to solidify into a cake; deriving the chemical mechanical polishing pad polishing layer from the cake; wherein the chemical mechanical polishing pad polishing layer has a polishing surface with the groove

(Continued)



pattern formed into the polishing surface; and wherein the polishing surface is adapted for polishing a substrate.

**9 Claims, 11 Drawing Sheets****(51) Int. Cl.**

*H01L 21/302* (2006.01)  
*H01L 21/00* (2006.01)

**(56) References Cited**

## U.S. PATENT DOCUMENTS

3,954,544 A 5/1976 Hooker  
4,053,283 A 10/1977 Schneider et al.  
4,144,295 A 3/1979 Dever, Jr.

|                   |         |                          |                        |
|-------------------|---------|--------------------------|------------------------|
| 5,110,081 A *     | 5/1992  | Lang, Jr. ....           | F16F 3/0873<br>248/635 |
| 5,163,584 A       | 11/1992 | Huber et al.             |                        |
| 7,214,757 B2 *    | 5/2007  | Gloyer .....             | C08G 18/10<br>528/60   |
| 7,670,517 B2      | 3/2010  | Tadokoro et al.          |                        |
| 8,314,029 B2      | 11/2012 | Hirose et al.            |                        |
| 9,457,449 B1      | 10/2016 | Brugarolas Brufau et al. |                        |
| 9,539,694 B1      | 1/2017  | Kozhukh et al.           |                        |
| 2006/0089095 A1 * | 4/2006  | Swisher .....            | B24B 37/205<br>451/533 |
| 2007/0128372 A1   | 6/2007  | Wirth et al.             |                        |
| 2009/0094900 A1   | 4/2009  | Swisher et al.           |                        |
| 2016/0037552 A1   | 2/2016  | Svedman et al.           |                        |
| 2016/0375543 A1   | 12/2016 | Qian et al.              |                        |
| 2016/0375545 A1   | 12/2016 | Qian et al.              |                        |
| 2016/0375550 A1   | 12/2016 | Tong et al.              |                        |
| 2016/0375553 A1   | 12/2016 | Veneziale et al.         |                        |
| 2016/0375554 A1   | 12/2016 | Qian et al.              |                        |
| 2016/0379840 A1   | 12/2016 | Qian et al.              |                        |

\* cited by examiner



Figure 1



Figure 2



Figure 3



Figure 4



Figure 5



Figure 6



Figure 7



Figure 8



Figure 9



Figure 10



Figure 11

**METHOD OF MAKING POLISHING LAYER  
FOR CHEMICAL MECHANICAL POLISHING  
PAD**

This application is a continuation-in-part of U.S. Ser. No. 14/751,423, filed Jun. 26, 2015, now pending.

The present invention relates to a method of forming a chemical mechanical polishing pad polishing layer. More particularly, the present invention relates to a method of forming a chemical mechanical polishing pad polishing layer using an axial mixing device.

In the fabrication of integrated circuits and other electronic devices, multiple layers of conducting, semiconducting and dielectric materials are deposited onto and removed from a surface of a semiconductor wafer. Thin layers of conducting, semiconducting and dielectric materials may be deposited using a number of deposition techniques. Common deposition techniques in modern wafer processing include physical vapor deposition (PVD), also known as sputtering, chemical vapor deposition (CVD), plasma-enhanced chemical vapor deposition (PECVD) and electro-chemical plating, among others. Common removal techniques include wet and dry isotropic and anisotropic etching, among others.

As layers of materials are sequentially deposited and removed, the uppermost surface of the wafer becomes non-planar. Because subsequent semiconductor processing (e.g., metallization) requires the wafer to have a flat surface, the wafer needs to be planarized. Planarization is useful for removing undesired surface topography and surface defects, such as rough surfaces, agglomerated materials, crystal lattice damage, scratches and contaminated layers or materials.

Chemical mechanical planarization, or chemical mechanical polishing (CMP), is a common technique used to planarize or polish work pieces such as semiconductor wafers. In conventional CMP, a wafer carrier, or polishing head, is mounted on a carrier assembly. The polishing head holds the wafer and positions the wafer in contact with a polishing layer of a polishing pad that is mounted on a table or platen within a CMP apparatus. The carrier assembly provides a controllable pressure between the wafer and polishing pad. Simultaneously, a polishing medium (e.g., slurry) is dispensed onto the polishing pad and is drawn into the gap between the wafer and polishing layer. To effect polishing, the polishing pad and wafer typically rotate relative to one another. As the polishing pad rotates beneath the wafer, the wafer sweeps out a typically annular polishing track, or polishing region, wherein the wafer's surface directly confronts the polishing layer. The wafer surface is polished and made planar by chemical and mechanical action of the polishing layer and polishing medium on the surface.

Hirose et al. disclose a method of making polishing layers in U.S. Pat. No. 8,314,029. Specifically, Hirose et al. disclose a method for manufacturing a polishing pad containing substantially spherical cells and having high thickness accuracy, which includes preparing a cell dispersed urethane composition by a mechanical foaming method; continuously discharging the cell dispersed urethane composition from a single discharge port to a substantially central portion in the width direction of a face material A, while feeding the face material A; laminating a face material B on the cell dispersed urethane composition; then uniformly adjusting the thickness of the cell dispersed urethane composition by thickness adjusting means; curing the cell dispersed urethane composition with the thickness adjusted in the preceding step

without applying any additional load to the composition so that a polishing sheet including a polyurethane foam is formed; and cutting the polishing sheet.

Notwithstanding, there is a continuing need for improved methods of manufacturing polishing layers for chemical mechanical polishing pads. Particularly for methods that reduce the total number of process steps required to provide the completed polishing pad. Hence, what is needed is an improved method of providing a polishing layer for a chemical mechanical polishing pad.

The present invention provides a method of forming a chemical mechanical polishing pad polishing layer, comprising: providing a mold having a base, wherein the base has a negative of a groove pattern formed therein; providing a poly side (P) liquid component, comprising at least one of a (P) side polyol, a (P) side polyamine and a (P) side alcohol amine; providing an iso side (I) liquid component, comprising at least one polyfunctional isocyanate; providing a pressurized gas; providing an axial mixing device having an internal cylindrical chamber; wherein the internal cylindrical chamber has a closed end, an open end, an axis of symmetry, at least one (P) side liquid feed port that opens into the internal cylindrical chamber, at least one (I) side liquid feed port that opens into the internal cylindrical chamber, and at least one tangential pressurized gas feed port that opens into the internal cylindrical chamber; wherein the closed end and the open end are perpendicular to the axis of symmetry; wherein the at least one (P) side liquid feed port and the at least one (I) side liquid feed port are arranged along a circumference of the internal cylindrical chamber proximate the closed end; wherein the at least one tangential pressurized gas feed port is arranged along the circumference of the internal cylindrical chamber downstream of the at least one (P) side liquid feed port and the at least one (I) side liquid feed port from the closed end; wherein the poly side (P) liquid component is introduced into the internal cylindrical chamber through the at least one (P) side liquid feed port at a (P) side charge pressure of 6,895 to 27,600 kPa; wherein the iso side (I) liquid component is introduced into the internal cylindrical chamber through the at least one (I) side liquid feed port at an (I) side charge pressure of 6,895 to 27,600 kPa; wherein a combined mass flow rate of the poly side (P) liquid component and the iso side (I) liquid component to the internal cylindrical chamber is 1 to 500 g/s, such as, preferably, from 2 to 40 g/s or, more preferably, 2 to 25 g/s; wherein the poly side (P) liquid component, the iso side (I) liquid component and the pressurized gas are intermixed within the internal cylindrical chamber to form a combination; wherein the pressurized gas is introduced into the internal cylindrical chamber through the at least one tangential pressurized gas feed port with a supply pressure of 150 to 1,500 kPa; wherein an inlet velocity into the internal cylindrical chamber of the pressurized gas is 50 to 600 m/s calculated based on ideal gas conditions at 20° C. and 1 atm pressure, or, preferably, 75 to 350 m/s; discharging the combination from the open end of the internal cylindrical chamber toward the base at a velocity of 5 to 1,000 m/sec, or, preferably, from 10 to 600 m/sec or, more preferably, from 15 to 450 m/sec; allowing the combination to solidify into a cake; separating the cake from the mold; and deriving the chemical mechanical polishing pad polishing layer from the cake; wherein the chemical mechanical polishing pad polishing layer has a polishing surface with the groove pattern formed into the polishing surface and wherein the polishing surface is adapted for polishing a substrate.

## BRIEF DESCRIPTION OF THE DRAWINGS

FIG. 1 is a depiction of a perspective view of a mold for use in the method of the present invention.

FIG. 2 is a depiction of a side elevational view of an axial mixing device for use in the method of the present invention.

FIG. 3 is a cross sectional view taken along line A-A in FIG. 2.

FIG. 4 is a depiction of a side elevational view of a chemical mechanical polishing pad polishing layer formed in a mold of the present invention.

FIG. 5 is a depiction of a perspective view of a chemical mechanical polishing pad polishing layer of the present invention.

FIG. 6 is a depiction of a top plan view of a groove pattern formed in the polishing surface of a chemical mechanical polishing pad polishing layer.

FIG. 7 is a depiction of a top plan view of a groove pattern formed in the polishing surface of a chemical mechanical polishing pad polishing layer.

FIG. 8 is a cross section view taken along line C-C in FIG. 7.

FIG. 9 is a depiction of a top plan view of a groove pattern formed in the polishing surface of a chemical mechanical polishing pad polishing layer.

FIG. 10 is a depiction of a top plan view of a groove pattern formed in the polishing surface of a chemical mechanical polishing pad polishing layer.

FIG. 11 is a cross sectional view taken along line B-B in FIG. 2.

## DETAILED DESCRIPTION

Various conventional processes for forming chemical mechanical polishing layers, such as, casting processes (i.e., forming cakes to be skived into multiple polishing layers) and frothing require sufficiently long gel times to facilitate the processing. Both frothing and casting processes require machining of the final groove pattern into the surface of the polishing layers formed. The method of the present invention greatly enhances the quality of the groove pattern formed in the polishing surface of the polishing layer and eliminates the need for machining the groove pattern into the finished polishing layer as is required by many conventional polishing layer manufacturing methods. The method of the present invention also enables a broader compositional window than would be suitable for conventional polishing layer manufacturing processes given the inherent limitations in the conventional techniques (i.e., gel time constraints).

The term “substantially circular cross section” as used herein and in the appended claims in reference to a mold cavity (20) means that the longest radius,  $r_c$ , of the mold cavity (20) projected onto the x-y plane (30) from the mold cavity's central axis,  $C_{axis}$ , (22) to a vertical internal boundary (18) of a surrounding wall (15) is  $\leq 20\%$  longer than the shortest radius,  $r_c$ , of the mold cavity (20) projected onto the x-y plane (30) from the mold cavity's central axis,  $C_{axis}$ , (22) to the vertical internal boundary (18). (See FIG. 1).

The term “mold cavity” as used herein and in the appended claims refers to the volume defined by a base (12) and a vertical internal boundary (18) of a surrounding wall (15). (See FIGS. 1 and 4).

The term “substantially perpendicular” as used herein and in the appended claims in reference to a first feature (e.g., a horizontal internal boundary; a vertical internal boundary)

relative to a second feature (e.g., an axis, an x-y plane) means that the first feature is at an angle of 80 to 100° to the second feature.

The term “essentially perpendicular” as used herein and in the appended claims in reference to a first feature (e.g., a horizontal internal boundary; a vertical internal boundary) relative to a second feature (e.g., an axis, an x-y plane) means that the first feature is at an angle of 85 to 95° to the second feature.

10 The term “average thickness,  $T_{P-avg}$ ” as used herein and in the appended claims in reference to a chemical mechanical polishing pad polishing layer (90) having a polishing surface (95) means the average thickness,  $T_P$ , of the chemical mechanical polishing pad polishing layer in a direction normal to the polishing surface (95) from the polishing surface (95) to the bottom surface (92) of the chemical mechanical polishing pad polishing layer (90). (See FIG. 5).

The term “substantially circular cross section” as used herein and in the appended claims in reference to a chemical mechanical polishing pad polishing layer (90) means that the longest radius,  $r_p$ , of the cross section from the central axis (98) of the chemical mechanical polishing pad polishing layer (90) to the outer perimeter (110) of the polishing surface (95) of the chemical mechanical polishing pad polishing layer (90) is  $\leq 20\%$  longer than the shortest radius,  $r_p$ , of the cross section from the central axis (98) to the outer perimeter (110) of the polishing surface (95). (See FIG. 5).

The chemical mechanical polishing pad polishing layer (90) of the present invention is preferably adapted for 20 rotation about a central axis (98). (See FIG. 5). Preferably, the polishing surface (95) of the chemical mechanical polishing pad polishing layer (90) is in a plane (99) perpendicular to the central axis (98). Preferably, the chemical mechanical polishing pad polishing layer (90) is adapted for 25 rotation in a plane (99) that is at an angle,  $\gamma$ , of 85 to 95° to the central axis (98), preferably, of 90° to the central axis (98). Preferably, the chemical mechanical polishing pad polishing layer (90) has a polishing surface (95) that has a substantially circular cross section perpendicular to the 30 central axis (98). Preferably, the radius,  $r_p$ , of the cross section of the polishing surface (95) perpendicular to the central axis (98) varies by  $\leq 20\%$  for the cross section, more preferably by  $\leq 10\%$  for the cross section.

The term “gel time” as used herein and in the appended 35 claims in reference to a combination of a poly side (P) liquid component and an iso side (I) liquid component formed in an axial mixing device of the present invention, means the total cure time for that combination determined using a standard test method according to ASTM D3795-00a (Reapproved 2006)(*Standard Test Method for Thermal Flow, Cure, and Behavior Properties of Pourable Thermosetting Materials by Torque Rheometer*).

The term “poly(urethane)” as used herein and in the appended claims encompasses (a) polyurethanes formed 45 from the reaction of (i) isocyanates and (ii) polyols (including diols); and, (b) poly(urethane) formed from the reaction of (i) isocyanates with (ii) polyols (including diols) and (iii) water, amines or a combination of water and amines.

50 Preferably, the method of forming a chemical mechanical polishing pad polishing layer of the present invention, comprises: providing a mold (10) having a base (12), wherein the base (12) of the mold (10) has a negative (14) of a groove pattern (100) formed therein; providing a poly side (P) liquid component, comprising at least one of a (P) side polyol, a (P) side polyamine and a (P) side alcohol amine; providing an iso side (I) liquid component, comprising 55 at least one polyfunctional isocyanate; providing a

pressurized gas; providing an axial mixing device (60) having an internal cylindrical chamber (65); wherein the internal cylindrical chamber (65) has a closed end (62), an open end (68), an axis of symmetry (70), at least one (P) side liquid feed port (75) that opens into the internal cylindrical chamber (65), at least one (I) side liquid feed port (80) that opens into the internal cylindrical chamber (65), and at least one (preferably, at least two) tangential pressurized gas feed port (85) that opens into the internal cylindrical chamber (65); wherein the closed end (62) and the open end (68) are perpendicular to the axis of symmetry (70) of the internal cylindrical chamber (65); wherein the at least one (P) side liquid feed port (75) and the at least one (I) side liquid feed port (80) are arranged along a circumference (67) of the internal cylindrical chamber (65) proximate the closed end (62); wherein the at least one (preferably, at least two) tangential pressurized gas feed port (85) is arranged along the circumference (67) of the internal cylindrical chamber (65) downstream of the at least one (P) side liquid feed port (75) and the at least one (I) side liquid feed port (80) from the closed end (62); wherein the poly side (P) liquid component is introduced into the internal cylindrical chamber (65) through the at least one (P) side liquid feed port (75) at a (P) side charge pressure of 6,895 to 27,600 kPa; wherein the iso side (I) liquid component is introduced into the internal cylindrical chamber (65) through the at least one (I) side liquid feed port (80) at an (I) side charge pressure of 6,895 to 27,600 kPa; wherein a combined mass flow rate of the poly side (P) liquid component and the iso side (I) liquid component to the internal cylindrical chamber (65) is 1 to 500 g/s (preferably, 2 to 40 g/s; more preferably 2 to 25 g/s); wherein the poly side (P) liquid component, the iso side (I) liquid component and the pressurized gas are intermixed within the internal cylindrical chamber (65) to form a combination; wherein the pressurized gas is introduced into the internal cylindrical chamber (65) through the at least one (preferably, at least two) tangential pressurized gas feed port (85) with a supply pressure of 150 to 1,500 kPa; wherein an inlet velocity into the internal cylindrical chamber (65) of the pressurized gas is 50 to 600 m/s calculated based on ideal gas conditions at 20° C. and 1 atm pressure, or, preferably, 75 to 350 m/s; discharging the combination from the open end (68) of the internal cylindrical chamber (65) toward the base (12) of the mold (10) at a velocity of 5 to 1,000 m/sec, or, preferably, from 10 to 600 m/sec or, more preferably, from 15 to 450 m/sec; allowing the combination to solidify into a cake; separating the cake from the mold (10); and, deriving the chemical mechanical polishing pad polishing layer (90) from the cake, wherein the chemical mechanical polishing pad polishing layer (90) has a polishing surface (95) with the groove pattern (100) formed into the polishing surface (95), and wherein the polishing surface (95) is adapted for polishing a substrate.

Preferably, the base (12) of the mold (10) used in the method of the present invention defines a negative (14) of a groove pattern; wherein the groove pattern (100) is transferred to the polishing surface (95) of the chemical mechanical polishing pad polishing layer (90). Preferably, the base (12) of the mold (10) has a substantially circular cross section having an average radius,  $r_c$ , (preferably, wherein  $r_c$  is 20 to 100 cm; more preferably, wherein  $r_c$  is 25 to 65 cm; most preferably, wherein  $r_c$  is 40 to 60 cm). (See FIGS. 1 and 4).

Preferably, the mold (10) used in the method of the present invention can have a surrounding wall (15). Preferably, the surrounding wall defines a vertical internal boundary (18) of the mold cavity (20) that is substantially per-

pendicular to the x-y plane (30). More preferably, the surrounding wall defines an vertical internal boundary (18) of the mold cavity (20) that is essentially perpendicular to the x-y plane (30). (See FIGS. 1 and 4).

Preferably, the mold cavity (20) has a central axis,  $C_{axis}$ , (22) that coincides with the z-axis and that intersects the horizontal internal boundary (14) of the base (12) of the mold (10) at a center point (21). Preferably, the center point (21) is located at the geometric center of the cross section,  $C_{x-sect}$ , (24) of the mold cavity (20) projected onto the x-y plane (30). (See FIG. 1).

Preferably, the mold cavity's cross section,  $C_{x-sect}$ , (24) projected onto the x-y plane (30) can be any regular or irregular two dimensional shape. Preferably, the mold cavity's cross section,  $C_{x-sect}$ , (24) is selected from a polygon and an ellipse. More preferably, the mold cavity's cross section,  $C_{x-sect}$ , (24) is a substantially circular cross section having an average radius,  $r_c$ , (preferably, wherein  $r_c$  is 20 to 100 cm; more preferably, wherein  $r_c$  is 25 to 65 cm; most preferably, wherein  $r_c$  is 40 to 60 cm). Most preferably, the mold cavity (20) approximates a right cylindrically shaped region having a substantially circular cross section,  $C_{x-sect}$ ; wherein the mold cavity has an axis of symmetry,  $C_{x-sym}$ , (25) which coincides with the mold cavity's central axis,  $C_{axis}$ , (22); wherein the right cylindrically shaped region has a cross sectional area,  $C_{x-area}$ , defined as follows:

$$C_{x-area} = \pi r_c^2$$

wherein  $r_c$  is the average radius of the mold cavity's cross sectional area,  $C_{x-area}$ , projected onto the x-y plane (30); and wherein  $r_c$  is 20 to 100 cm (more preferably, 25 to 65 cm; most preferably, 40 to 60 cm). (See FIGS. 1 and 4).

Preferably, the axial mixing device (60) used in the method of the present invention has an internal cylindrical chamber (65). Preferably, the internal cylindrical chamber (65) has a closed end (62) and an open end (68). Preferably, the closed end (62) and the open end (68) are each substantially perpendicular to an axis of symmetry (70) of the internal cylindrical chamber (65). More preferably, the closed end (62) and the open end (68) are each essentially perpendicular to an axis of symmetry (70) of the internal cylindrical chamber (65). Most preferably, the closed end (62) and the open end (68) are each perpendicular to an axis of symmetry (70) of the internal cylindrical chamber (65). (See FIGS. 2-3 and 11).

Preferably, the axial mixing device (60) used in the method of the present invention has an internal cylindrical chamber (65) with an axis of symmetry (70), wherein the open end (68) has a circular opening (69). More preferably, the axial mixing device (60) used in the method of the present invention has an internal cylindrical chamber (65) with an axis of symmetry (70); wherein the open end (68) has a circular opening (69); and, wherein the circular opening (69) is concentric with the internal cylindrical chamber (65). Most preferably, the axial mixing device (60) used in the method of the present invention has an internal cylindrical chamber (65) with an axis of symmetry (70); wherein the open end (68) has a circular opening (69); wherein the circular opening (69) is concentric with the internal cylindrical chamber (65); and, wherein the circular opening (69) is perpendicular to the axis of symmetry (70) of the internal cylindrical chamber (65). Preferably, the circular opening (69) has a diameter of 1 to 10 mm (more preferably, 1.5 to 7.5 mm; still more preferably 2 to 6 mm; most preferably, 2.5 to 3.5 mm). (See FIGS. 2-3 and 11).

Preferably, the axial mixing device (60) used in the method of the present invention has at least one (P) side



arranged along the circumference of the internal cylindrical chamber (65) downstream of the at least one (P) side liquid feed port (75) and the at least one (I) side liquid feed port (80) from the closed end (62). Still more preferably, the axial mixing device (60) used in the method of the present invention has at least two tangential pressurized gas feed ports (85) that open into the internal cylindrical chamber (65); wherein the at least two tangential pressurized gas feed ports (85) are arranged along the circumference of the internal cylindrical chamber (65) downstream of the at least one (P) side liquid feed port (75) and the at least one (I) side liquid feed port (80) from the closed end (62). Yet still more preferably, the axial mixing device (60) used in the method of the present invention has at least two tangential pressurized gas feed ports (85) that open into the internal cylindrical chamber (65); wherein the at least two tangential pressurized gas feed ports (85) are arranged along the circumference of the internal cylindrical chamber (65) downstream of the at least one (P) side liquid feed port (75) and the at least one (I) side liquid feed port (80) from the closed end (62); and, wherein the at least two tangential pressurized gas feed ports (85) are arranged evenly about a circumference (67) of the internal cylindrical chamber (65). Most preferably, the axial mixing device (60) used in the method of the present invention has at least two tangential pressurized gas feed ports (85) that open into the internal cylindrical chamber (65); wherein the at least two tangential pressurized gas feed ports (85) are arranged along the circumference of the internal cylindrical chamber (65) downstream of the at least one (P) side liquid feed port (75) and the at least one (I) side liquid feed port (80) from the closed end (62); and, wherein the at least two tangential pressurized gas feed ports (85) are arranged evenly about a circumference (67) of the internal cylindrical chamber (65) and are at an equal distance from the closed end (62) of the internal cylindrical chamber (65). Preferably, the at least one tangential pressurized gas feed port opens into the internal cylindrical chamber (65) through an orifice having a critical dimension of 0.1 to 5 mm (preferably, 0.3 to 3 mm; more preferably, 0.5 to 2 mm). Preferably, the at least one tangential pressurized gas feed port opens into the internal cylindrical chamber (65) and is directed tangentially along an internal circumference of the internal cylindrical chamber (65). More preferably, the at least one tangential pressurized gas feed port opens into the internal cylindrical chamber (65) and is directed tangentially along an internal circumference of the internal cylindrical chamber and on a plane that is essentially perpendicular to the axis of symmetry (70) of the internal cylindrical chamber (65). Most preferably, the at least one tangential pressurized gas feed port opens into the internal cylindrical chamber (65) and is directed tangentially along an internal circumference of the internal cylindrical chamber and on a plane that is perpendicular to the axis of symmetry (70) of the internal cylindrical chamber (65).

Preferably, in the method of the present invention, the poly side (P) liquid component, comprises at least one of a (P) side polyol, a (P) side polyamine and a (P) side alcohol amine.

Preferably, the (P) side polyol is selected from the group consisting of diols, polyols, polyol diols, copolymers thereof and mixtures thereof. More preferably, the (P) side polyol is selected from the group consisting of polyether polyols (e.g., poly(oxytetramethylene)glycol, poly(oxypropylene)glycol and mixtures thereof); polycarbonate polyols; polyester polyols; polycaprolactone polyols; mixtures thereof; and, mixtures thereof with one or more low molecular weight polyols selected from the group consisting of ethylene

glycol; 1,2-propylene glycol; 1,3-propylene glycol; 1,2-butanediol; 1,3-butanediol; 2-methyl-1,3-propanediol; 1,4-butanediol; neopentyl glycol; 1,5-pentanediol; 3-methyl-1,5-pentanediol; 1,6-hexanediol; diethylene glycol; dipropylene glycol; and, tripropylene glycol. Still more preferably, the at least one (P) side polyol is selected from the group consisting of polytetramethylene ether glycol (PTMEG); ester based polyols (such as ethylene adipates, butylene adipates); polypropylene ether glycols (PPG); polycaprolactone polyols; copolymers thereof; and, mixtures thereof. Preferably, the poly side (P) liquid component comprises 25 to 95 wt % of a (P) side polyol.

Preferably, in the method of the present invention, the poly side (P) liquid component used contains at least one (P) side polyol; wherein the at least one (P) side polyol includes a high molecular weight polyol having a number average molecular weight,  $M_N$ , of 2,500 to 100,000. More preferably, the high molecular weight polyol used has a number average molecular weight,  $M_N$ , of 5,000 to 50,000 (still more preferably 7,500 to 25,000; most preferably 10,000 to 12,000).

Preferably, in the method of the present invention, the poly side (P) liquid component used contains at least one (P) side polyol; wherein the at least one (P) side polyol includes a high molecular weight polyol having an average of three to ten hydroxyl groups per molecule. More preferably, the high molecular weight polyol used has an average of four to eight (still more preferably five to seven; most preferably six) hydroxyl groups per molecule.

Examples of commercially available high molecular weight polyols include Specflex® polyols, Voranol® polyols and Voralux® polyols (available from The Dow Chemical Company); Multranol® Specialty Polyols and Ultracel® Flexible Polyols (available from Bayer MaterialScience LLC); and Pluracol® Polyols (available from BASF). A number of preferred high molecular weight polyols are listed in TABLE 1.

TABLE 1

| High molecular weight polyol | Number of OH groups per molecule | $M_N$  | Hydroxyl Number (mg KOH/g) |
|------------------------------|----------------------------------|--------|----------------------------|
| Multranol ® 3901 Polyol      | 3.0                              | 6,000  | 28                         |
| Pluracol ® 1385 Polyol       | 3.0                              | 3,200  | 50                         |
| Pluracol ® 380 Polyol        | 3.0                              | 6,500  | 25                         |
| Pluracol ® 1123 Polyol       | 3.0                              | 7,000  | 24                         |
| ULTRACEL ® 3000 Polyol       | 4.0                              | 7,500  | 30                         |
| SPECFLEX ® NC630 Polyol      | 4.2                              | 7,602  | 31                         |
| SPECFLEX ® NC632 Polyol      | 4.7                              | 8,225  | 32                         |
| VORALUX ® HF 505 Polyol      | 6.0                              | 11,400 | 30                         |
| MULTRANOL ® 9185 Polyol      | 6.0                              | 3,366  | 100                        |
| VORANOL ® 4053 Polyol        | 6.9                              | 12,420 | 31                         |

Preferably, the (P) side polyamine is selected from the group consisting of diamines and other multifunctional amines. More preferably, the (P) side polyamine is selected from the group consisting of aromatic diamines and other multifunctional aromatic amines; such as, for example, 4,4'-methylene-bis-o-chloroaniline ("MbOCA"); 4,4'-methylene-bis-(3-chloro-2,6-diethylaniline) ("MCDEA"); dimethylthiotoluenediamine; trimethyleneglycol di-p-aminobenzoate; polytetramethyleneoxide mono-p-aminobenzoate; polytetramethyleneoxide mono-p-aminobenzoate; polypropyleneoxide di-p-aminobenzoate; polypropyleneoxide mono-p-aminobenzoate; 1,2-bis(2-aminophenylthio)ethane; 4,4'-methylene-bis-aniline; diethyltoluenediamine; 5-tert-butyl-2,4-toluendiamine; 3-tert-butyl-2,6-toluenediamine;

## 11

5-tert-amyl-2,4-toluenediamine; and 3-tert-amyl-2,6-toluenediamine and chlorotoluenediamine.

Preferably, the (P) side alcohol amine is selected from the group consisting amine initiated polyols. More preferably, the (P) side alcohol amine is selected from the group consisting amine initiated polyols containing one to four (still more preferably, two to four; most preferably, two) nitrogen atoms per molecule. Preferably, the (P) side alcohol amine is selected from the group consisting amine initiated polyols that have an average of at least three hydroxyl groups per molecule. More preferably, the (P) side alcohol amine is selected from the group consisting of amine initiated polyols that have an average of three to six (still more preferably, three to five; most preferably, four) hydroxyl groups per molecule. Particularly preferred amine initiated polyols a number average molecular weight,  $M_N$ , of  $\leq 700$  (preferably, of 150 to 650; more preferably, of 200 to 500; most preferably 250 to 300) and have a hydroxyl number (as determined by ASTM Test Method D4274-11) of 350 to 1,200 mg KOH/g. More preferably, the amine initiated polyol used has a hydroxyl number of 400 to 1,000 mg KOH/g (most preferably 600 to 850 mg KOH/g). Examples of commercially available amine initiated polyols include the Voranol® family of amine initiated polyols (available from The Dow Chemical Company); the Quadrol® Specialty Polyols (N,N,N',N'-tetrakis(2-hydroxypropyl ethylene diamine)) (available from BASF); Pluracol® amine based polyols (available from BASF); Multranol® amine based polyols (available from Bayer MaterialScience LLC); triisopropanolamine (TIPA) (available from The Dow Chemical Company); and, triethanolamine (TEA) (available from Mallinckrodt Baker Inc.). A number of preferred amine initiated polyols are listed in TABLE 2.

TABLE 2

| Amine initiated polyol  | Number of OH groups per molecule | $M_N$ | Hydroxyl Number (mg KOH/g) |
|-------------------------|----------------------------------|-------|----------------------------|
| Triethanolamine         | 3                                | 149   | 1130                       |
| Triisopropanolamine     | 3                                | 192   | 877                        |
| MULTRANOL ® 9138 Polyol | 3                                | 240   | 700                        |
| MULTRANOL ® 9170 Polyol | 3                                | 481   | 350                        |
| VORANOL ® 391 Polyol    | 4                                | 568   | 391                        |
| VORANOL ® 640 Polyol    | 4                                | 352   | 638                        |
| VORANOL ® 800 Polyol    | 4                                | 280   | 801                        |
| QUADROL ® Polyol        | 4                                | 292   | 770                        |
| MULTRANOL ® 4050 Polyol | 4                                | 356   | 630                        |
| MULTRANOL ® 4063 Polyol | 4                                | 488   | 460                        |
| MULTRANOL ® 8114 Polyol | 4                                | 568   | 395                        |
| MULTRANOL ® 8120 Polyol | 4                                | 623   | 360                        |
| MULTRANOL ® 9181 Polyol | 4                                | 291   | 770                        |
| VORANOL ® 202 Polyol    | 5                                | 590   | 475                        |

Preferably, in the method of the present invention, the poly side (P) liquid component is introduced into the internal cylindrical chamber (65) through the at least one (P) side liquid feed port (75) at a (P) side charge pressure of 6,895 to 27,600 kPa. More preferably, the poly side (P) liquid component is introduced into the internal cylindrical chamber (65) through the at least one (P) side liquid feed port (75) at a (P) side charge pressure of 8,000 to 20,000 kPa. Most preferably, the poly side (P) liquid component is introduced into the internal cylindrical chamber (65) through the at least one (P) side liquid feed port (75) at a (P) side charge pressure of 10,000 to 17,000 kPa.

Preferably, in the method of the present invention, the iso side (I) liquid component, comprises at least one polyfunc-

## 12

tional isocyanate. Preferably, the at least one polyfunctional isocyanate contains two reactive isocyanate groups (i.e., NCO).

Preferably, the at least one polyfunctional isocyanate is selected from the group consisting of an aliphatic polyfunctional isocyanate, an aromatic polyfunctional isocyanate and a mixture thereof. More preferably, the polyfunctional isocyanate is a diisocyanate selected from the group consisting of 2,4-toluene diisocyanate; 2,6-toluene diisocyanate; 4,4'-diphenylmethane diisocyanate; naphthalene-1,5-diisocyanate; tolidine diisocyanate; para-phenylene diisocyanate; xylylene diisocyanate; isophorone diisocyanate; hexamethylene diisocyanate; 4,4'-dicyclohexylmethane diisocyanate; cyclohexanediisocyanate; and, mixtures thereof. Still more preferably, the at least one polyfunctional isocyanate is an isocyanate terminated urethane prepolymer formed by the reaction of a diisocyanate with a prepolymer polyol.

Preferably, the at least one polyfunctional isocyanate is an isocyanate-terminated urethane prepolymer; wherein the isocyanate-terminated urethane prepolymer has 2 to 12 wt % unreacted isocyanate (NCO) groups. More preferably, the isocyanate-terminated urethane prepolymer used in the method of the present invention has 2 to 10 wt % (still more preferably 4 to 8 wt %; most preferably 5 to 7 wt %) unreacted isocyanate (NCO) groups.

Preferably, the isocyanate terminated urethane prepolymer used is the reaction product of a diisocyanate with a prepolymer polyol; wherein the prepolymer polyol is selected from the group consisting of diols, polyols, polyol diols, copolymers thereof and mixtures thereof. More preferably, the prepolymer polyol is selected from the group consisting of polyether polyols (e.g., poly(oxytetramethylene)glycol, poly(oxypropylene)glycol and mixtures thereof); polycarbonate polyols; polyester polyols; polycaprolactone polyols; mixtures thereof; and, mixtures thereof with one or more low molecular weight polyols selected from the group consisting of ethylene glycol; 1,2-propylene glycol; 1,3-propylene glycol; 1,2-butanediol; 1,3-butanediol; 2-methyl-1,3-propanediol; 1,4-butanediol; neopentyl glycol; 1,5-pentanediol; 3-methyl-1,5-pentanediol; 1,6-hexanediol; diethylene glycol; dipropylene glycol; and, tripropylene glycol. Still more preferably, the prepolymer polyol is selected from the group consisting of polytetramethylene ether glycol (PTMEG); ester based polyols (such as ethylene adipates, butylene adipates); polypropylene ether glycols (PPG); polycaprolactone polyols; copolymers thereof and, mixtures thereof. Most preferably, the prepolymer polyol is selected from the group consisting of PTMEG and PPG.

Preferably, when the prepolymer polyol is PTMEG, the isocyanate terminated urethane prepolymer has an unreacted isocyanate (NCO) concentration of 2 to 10 wt % (more preferably of 4 to 8 wt %; most preferably 6 to 7 wt %). Examples of commercially available PTMEG based isocyanate terminated urethane prepolymers include Imuthane® prepolymers (available from COIM USA, Inc., such as, PET-80A, PET-85A, PET-90A, PET-93A, PET-95A, PET-60D, PET-70D, PET-75D); Adiprene® prepolymers (available from Chemtura, such as, LF 800A, LF 900A, LF 910A, LF 930A, LF 931A, LF 939A, LF 950A, LF 952A, LF 600D, LF 601D, LF 650D, LF 667, LF 700D, LF 750D, LF 751D, LF 752D, LF 753D and L325); Andur® prepolymers (available from Anderson Development Company, such as, 70APLF, 80APLF, 85APLF, 90APLF, 95APLF, 60DPLF, 70APLF, 75APLF).

Preferably, when the prepolymer polyol is PPG, the isocyanate terminated urethane prepolymer has an unreacted

isocyanate (NCO) concentration of 3 to 9 wt % (more preferably 4 to 8 wt %, most preferably 5 to 6 wt %). Examples of commercially available PPG based isocyanate terminated urethane prepolymers include Imuthane® prepolymers (available from COIM USA, Inc., such as, PPT-80A, PPT-90A, PPT-95A, PPT-65D, PPT-75D); Adiprene® prepolymers (available from Chemtura, such as, LFG 963A, LFG 964A, LFG 740D); and, Andur® prepolymers (available from Anderson Development Company, such as, 8000APLF, 9500APLF, 6500DPLF, 7501DPLF).

Preferably, the isocyanate terminated urethane prepolymer used in the method of the present invention is a low free isocyanate terminated urethane prepolymer having less than 0.1 wt % free toluene diisocyanate (TDI) monomer content.

Non-TDI based isocyanate terminated urethane prepolymers can also be used in the method of the present invention. For example, isocyanate terminated urethane prepolymers include those formed by the reaction of 4,4'-diphenylmethane diisocyanate (MDI) and polyols such as polytetramethylene glycol (PTMEG) with optional diols such as 1,4-butanediol (BDO) are acceptable. When such isocyanate terminated urethane prepolymers are used, the unreacted isocyanate (NCO) concentration is preferably 4 to 10 wt % (more preferably 4 to 8 wt %, most preferably 5 to 7 wt %). Examples of commercially available isocyanate terminated urethane prepolymers in this category include Imuthane® prepolymers (available from COIM USA, Inc. such as 27-85A, 27-90A, 27-95A); Andur® prepolymers (available from Anderson Development Company, such as, IE75AP, IE80AP, IE 85AP, IE90AP, IE95AP, IE98AP); Vibrathane® prepolymers (available from Chemtura, such as, B625, B635, B821); Isonate® modified prepolymer (available from The Dow Chemical Company, such as, Isonate® 240 with 18.7% NCO, Isonate® 181 with 23% NCO, Isonate® 143L with 29.2% NCO); and, polymeric MDI (available from The Dow Chemical Company, such as, PAPI® 20, 27, 94, 95, 580N, 901).

Preferably, in the method of the present invention, the iso side (I) liquid component is introduced into the internal cylindrical chamber (65) through the at least one (I) side liquid feed port (80) at an (I) side charge pressure of 6,895 to 27,600 kPa. More preferably, the iso side (I) liquid component is introduced into the internal cylindrical chamber (65) through the at least one (I) side liquid feed port (80) at an (I) side charge pressure of 8,000 to 20,000 kPa. Most preferably, the iso side (I) liquid component is introduced into the internal cylindrical chamber (65) through the at least one (I) side liquid feed port (80) at an (I) side charge pressure of 10,000 to 17,000 kPa.

Preferably, in the method of the present invention, at least one of the poly side (P) liquid component and the iso side (I) liquid component can optionally contain additional liquid materials. For example, at least one of the poly side (P) liquid component and the iso side (I) liquid component can contain liquid materials selected from the group consisting of foaming agents (e.g., carbamate foaming agents such as Specflex™ NR 556 CO<sub>2</sub>/aliphatic amine adduct available from The Dow Chemical Company); catalyst (e.g., tertiary amine catalysts such as Dabco® 33LV catalyst available from Air Products, Inc.; and tin catalyst such as Fomrez® tin catalyst from Momentive); and surfactants (e.g., Tegostab® silicon surfactant from Evonik). Preferably, in the method of the present invention, the poly side (P) liquid component contains an additional liquid material. More preferably, in the method of the present invention, the poly side (P) liquid component contains an additional liquid material; wherein the additional liquid material is at least one of a catalyst and

a surfactant. Most preferably, in the method of the present invention, the poly side (P) liquid component contains a catalyst and a surfactant.

Preferably, in the method of the present invention, the pressurized gas used is selected from the group consisting of carbon dioxide, nitrogen, air and argon. More preferably, the pressurized gas used is selected from the group consisting of carbon dioxide, nitrogen and air. Still more preferably, the pressurized gas used is selected from the group consisting of nitrogen and air. Most preferably, the pressurized gas used is air.

Preferably, in the method of the present invention, the pressurized gas used has a water content of  $\leq 10$  ppm. More preferably, the pressurized gas used has a water content of  $\leq 1$  ppm. Still more preferably, the pressurized gas used has a water content of  $\leq 0.1$  ppm. Most preferably, the pressurized gas used has a water content of  $\leq 0.01$  ppm.

Preferably, in the method of the present invention, the pressurized gas is introduced into the internal cylindrical chamber (65) through the at least two tangential pressurized gas feed ports (85) with an inlet velocity, wherein the inlet velocity is 90 to 600 m/s calculated based on ideal gas conditions at 20° C. and 1 atm pressure. Without wishing to be bound by theory, it is noted that when the inlet velocity is too low, the polishing layer deposited in the mold has an increased likelihood of developing undesirable cracks.

Preferably, in the method of the present invention, the pressurized gas is introduced into the internal cylindrical chamber (65) through the at least two tangential pressurized gas feed ports (85) with a supply pressure of 150 to 1,500 kPa. More preferably, the pressurized gas is introduced into the internal cylindrical chamber (65) through the at least two tangential pressurized gas feed ports (85) with a supply pressure of 350 to 1,000 kPa. Most preferably, the pressurized gas is introduced into the internal cylindrical chamber (65) through the at least two tangential pressurized gas feed ports (85) with a supply pressure of 550 to 830 kPa.

Preferably, the method of forming a chemical mechanical polishing pad polishing layer of the present invention, 40 comprises: providing a poly side (P) liquid component and an iso side (I) liquid component; wherein the poly side (P) liquid component and the iso side (I) liquid component are provided at a stoichiometric ratio of the reactive hydrogen groups (i.e., the sum of the amine (NH<sub>2</sub>) groups and the hydroxyl (OH) groups) in the components of the poly side (P) liquid component to the unreacted isocyanate (NCO) groups in the iso side (I) liquid component of 0.85 to 1.15 (more preferably 0.90 to 1.10; most preferably 0.95 to 1.05).

Preferably, in the method of the present invention, the 50 combined mass flow rate of the poly side (P) liquid component and the iso side (I) liquid component to the internal cylindrical chamber (65) is 1 to 500 g/s (preferably, 2 to 40 g/s; more preferably, 2 to 25 g/s).

Preferably, in the method of the present invention, the 55 ratio of (a) the sum of the combined mass flow rate of the poly side (P) liquid component and the iso side (I) liquid component to the internal cylindrical chamber (65) to (b) the mass flow of the pressurized gas to the internal cylindrical chamber (65) (calculated based on ideal gas conditions at 20° C. and 1 atm pressure) is  $\leq 46$  to 1 (more preferably,  $\leq 30$  to 1).

Preferably, in the method of the present invention, the 60 combination formed in the axial mixing device (60) is discharged from the open end (68) of the internal cylindrical chamber (65) toward the base (12) of the mold (10) at a velocity of 10 to 300 m/sec. More preferably, the combination is discharged from the opening (69) at the open end (68)

## 15

of the axial mixing device (60) with a velocity having a z-component in a direction parallel to the z axis (Z) toward the base (12) of the mold (10) of 10 to 300 m/sec.

Preferably, in the method of the present invention, the combination is discharged from the open end (68) of the axial mixing device (60) at a distance, D, along the z dimension from the bottom surface (92) of the chemical mechanical polishing pad polishing layer (90) formed in the mold (10). More preferably, the combination is discharged from the open end (68) of the axial mixing device (60) at a distance, D, along the z dimension from the bottom surface (92) of the chemical mechanical polishing pad polishing layer (90) formed in the mold (10); wherein the average distance,  $D_{avg}$ , is 2.5 to 125 cm (more preferably, 7.5 to 75 cm; most preferably, 12.5 to 50 cm).

Preferably, in the method of the present invention, the combination formed in the axial mixing device has a gel time of 5 to 900 seconds. More preferably, the combination formed in the axial mixing device has a gel time of 10 to 600 seconds. Most preferably, the combination formed in the axial mixing device has a gel time of 15 to 120 seconds.

Preferably, the chemical mechanical polishing pad polishing layer prepared using the method of the present invention can be interfaced with at least one additional layer to form a chemical mechanical polishing pad. Preferably, the chemical mechanical polishing pad polishing layer prepared using the method of the present invention is interfaced with a compressible subpad (not shown); wherein the compressible subpad is interfaced with the polishing layer (90) using a stack adhesive; wherein the stack adhesive is interposed between the bottom surface (92) of the polishing layer (90) and the compressible subpad. The subpad preferably improves conformance of the polishing layer to the surface of the substrate being polished. Preferably, the stack adhesive used is an adhesive selected from the group consisting of pressure sensitive adhesives, reactive hot melt adhesives, contact adhesives and combinations thereof. More preferably, the stack adhesive used is selected from the group consisting of reactive hot melt adhesives and pressure sensitive adhesives. Most preferably, the stack adhesive used is a reactive hot melt adhesive.

Preferably, the chemical mechanical polishing pad polishing layer prepared using the method of the present invention is incorporated into a chemical mechanical polishing pad, wherein the chemical mechanical polishing pad is adapted to be interfaced with the platen of a polishing machine. Preferably, the chemical mechanical polishing pad is adapted to be interfaced with the platen using at least one of a vacuum and a pressure sensitive platen adhesive.

Preferably, the chemical mechanical polishing pad polishing layer prepared using the method of the present invention is adapted for polishing a substrate; wherein the substrate is at least one of a magnetic substrate, an optical substrate and a semiconductor substrate. More preferably, the chemical mechanical polishing pad polishing layer prepared using the method of the present invention is adapted for polishing a substrate; wherein the substrate is a semiconductor substrate. Most preferably, the chemical mechanical polishing pad polishing layer prepared using the method of the present invention is adapted for polishing a substrate; wherein the substrate is a semiconductor wafer.

Preferably, in the method of the present invention, the chemical mechanical polishing pad polishing layer derived from the cake has a polishing surface with a groove pattern (100) formed into the polishing surface (95). Preferably, the groove pattern comprises one or more grooves arranged on the polishing surface such that upon rotation of the chemical

## 16

mechanical polishing pad polishing layer during polishing, the one or more grooves sweep over the surface of the substrate being polished. Preferably, the one or more grooves consist of curved grooves, linear grooves and combinations thereof.

Preferably, the groove pattern comprises a plurality of grooves. More preferably, the groove pattern is selected from a groove design. Preferably, the groove design is selected from the group consisting of concentric grooves (10) (which may be circular or spiral), curved grooves, cross hatch grooves (e.g., arranged as an X-Y grid across the pad surface), other regular designs (e.g., hexagons, triangles), tire tread type patterns, irregular designs (e.g., fractal patterns), and combinations thereof. More preferably, the groove design is selected from the group consisting of random grooves, concentric grooves, spiral grooves, cross-hatched grooves, X-Y grid grooves, hexagonal grooves, triangular grooves, fractal grooves and combinations thereof. Most preferably, the polishing surface has a spiral groove pattern formed therein. The groove profile is preferably selected from rectangular with straight side walls or the groove cross section may be "V" shaped, "U" shaped, saw-tooth, and combinations thereof.

Preferably, the groove pattern (100) comprises a plurality of grooves formed in the polishing surface (95) of a chemical mechanical polishing pad polishing layer (90), wherein the plurality of grooves are curved grooves (120). (See FIG. 6).

Preferably, the groove pattern (100) comprises a plurality of grooves formed in the polishing surface (95) of a chemical mechanical polishing pad polishing layer (90), wherein the plurality of grooves are concentric circular grooves (130). (See FIGS. 7-8).

Preferably, the groove pattern (100) comprises a plurality of grooves formed in the polishing surface (95) of a chemical mechanical polishing pad polishing layer (90), wherein the plurality of grooves are linear X-Y grooves (140). (See FIG. 9).

Preferably, the groove pattern (100) comprises a plurality of grooves formed in the polishing surface (95) of a chemical mechanical polishing pad layer (90), wherein the plurality of grooves comprise concentric circular grooves (130) and linear X-Y grooves (140). (See FIG. 10).

Preferably, the chemical mechanical polishing pad polishing layer (90) prepared using the method of the present invention has an average thickness,  $T_{P-avg}$ , of 20 to 150 mils. More preferably the chemical mechanical polishing pad polishing layer (90) prepared using the method of the present invention has an average thickness,  $T_{P-avg}$ , of 30 to 125 mils (still more preferably 40 to 120 mils; most preferably 50 to 100 mils). (See FIG. 5).

Some embodiments of the present invention will now be described in detail in the following Examples.

55 Example 1: Chemical Mechanical Polishing Pad  
Polishing Layer

A poly side (P) liquid component was provided, containing: 77.62 wt % high molecular weight polyether polyol (Voralux® HF 505 polyol available from The Dow Chemical Company); 21.0 wt % monoethylene glycol; 1.23 wt % of a silicone surfactant (Tegostab® B8418 surfactant available from Evonik); 0.05 wt % of a tin catalyst (Fomrez® UL-28 available from Momentive); and, 0.10 wt % of a tertiary amine catalyst (Dabco® 33LV catalyst available from Air Products, Inc.). An iso side (I) liquid component was provided, containing: 100 wt % of a modified diphe-

## 17

nylmethane diisocyanate (Isonate<sup>TM</sup> 181 MDI prepolymer available from The Dow Chemical Company.) A pressurized gas (dry air) was provided.

An axial mixing device was provided (a MicroLine 45 CSM available from Hennecke GmbH) having a (P) side liquid feed port, an (I) side liquid feed port and four tangential pressurized gas feed ports. The poly side (P) liquid component and the iso side (I) liquid component were fed to the axial mixing device through their respective feed ports with a (P) side charge pressure of 10,500 kPa, an (I) side charge pressure of 14,600 kPa and at a weight ratio of (I)/(P) of 1.36 (giving a stoichiometric ratio of reactive hydrogen groups to NCO groups of 0.95). The pressurized gas was fed through the tangential pressurized gas feed ports with a supply pressure of 830 kPa to give a combined liquid component to gas mass flow rate ratio through the axial mixing device of 3.7 to 1 to form a combination. The combination was discharged from the axial mixing device toward a mold base having a negative of a groove pattern formed therein (a negative K7 type pattern of concentric circular grooves) at a velocity of 254 m/sec to form a cake on the mold base. The cake was allowed to cure for 16 hours at 100° C. The cake was then allowed to cool to room temperature before separating it from the mold base. The bottom surface of the cake was machined flat on a lathe to provide a polishing layer. The polishing layer was then mated to a Suba IV subpad using a hot melt adhesive to provide a chemical mechanical polishing pad with a chemical mechanical polishing layer having a K7 type groove pattern (concentric circular grooves 20 mil wide, 30 mil deep and 70 mil pitch).

The polishing layer from and Example 1 was analyzed to determine its physical properties as reported in TABLE 3. Note that the density data reported were determined according to ASTM D1622; the Shore D hardness data reported were determined according to ASTM D2240; and, the elongation to break data reported were determined according to ASTM D412. Reported values for the physical properties of IC1000<sup>TM</sup> polishing layer material is also reported in TABLE 3 for comparison purposes.

TABLE 3

| Property                     | Example |       |
|------------------------------|---------|-------|
|                              | Ex. C1  | Ex. 1 |
| Density (g/cm <sup>3</sup> ) | 0.76    | 0.72  |
| Shore D Hardness, @ 2 s      | 56      | 48    |
| G'-40° C. (MPa)              | 118     | 77    |
| G''-40° C. (MPa)             | 11.0    | 8.8   |
| G'-30° C./G'-90° C.          | 3.6     | 2.7   |
| Tensile strength (MPa)       | 22      | 14    |
| Elongation to break (%)      | 124     | 171   |
| Tensile modulus (MPa)        | 260.0   | 113.5 |
| Toughness (MPa)              | 23.7    | 19.4  |

Comparative Example PC1 and Example P1

Chemical Mechanical Polishing Removal Rate Experiments

Silicon dioxide removal rate polishing tests were performed using the chemical mechanical polishing pad prepared according to Example 1 and compared with those obtained in Comparative Example PC1 using an IC1000<sup>TM</sup> polyurethane polishing pad with K7 grooves (commercially available from Rohm and Haas Electronic Materials CMP

## 18

Inc.). Specifically, the silicon dioxide removal rate for each of the polishing pads is provided in TABLE 4. The polishing removal rate experiments were performed on 200 mm blanket S15KTEN TEOS sheet wafers from Novellus Systems, Inc. An Applied Materials 200 mm Mirra<sup>®</sup> polisher was used. All polishing experiments were performed with a down force of 20.7 kPa (3 psi), a slurry flow rate of 200 ml/min (Klebosol<sup>TM</sup> 1730 slurry available from Rohm and Haas Electronic Materials CMP Inc.), a table rotation speed of 93 rpm and a carrier rotation speed of 87 rpm. A Saesol 8031C diamond pad conditioner (commercially available from Saesol Diamond Ind. Co., Ltd.) was used to condition the polishing pads. The polishing pads were each broken in with the conditioner using a down force of 31.1 N for 30 minutes. The polishing pads were further conditioned 100% in situ during polishing at 10 sweeps/min from 1.7 to 9.2 in from the center of the polishing pad with a down force of 31.1 N. The removal rates were determined by measuring the film thickness before and after polishing using a KLA-Tencor FX200 metrology tool using a 49 point spiral scan with a 3 mm edge exclusion. Each of the removal rate experiments were performed three times. The average removal rate for the triplicate removal rate experiments for each of the polishing pads is provided in TABLE 4.

TABLE 4

| Ex # | Chemical mechanical polishing pad    | TEOS removal rate (Å/min) |
|------|--------------------------------------|---------------------------|
| PC1  | IC1000 <sup>TM</sup> pad w/K7 groove | 2460                      |
| P1   | Ex. 1                                | 2850                      |

We claim:

1. A method of forming a chemical mechanical polishing pad polishing layer, comprising:
  - providing a mold having a base, wherein the base has a negative of a groove pattern formed therein;
  - providing a poly side (P) liquid component, comprising at least one of a (P) side polyol, a (P) side polyamine and a (P) side alcohol amine;
  - providing an iso side (I) liquid component, comprising at least one polyfunctional isocyanate;
  - providing a pressurized gas;
  - providing an axial mixing device having an internal cylindrical chamber, wherein the internal cylindrical chamber has a closed end, an open end, an axis of symmetry, at least one (P) side liquid feed port that opens into the internal cylindrical chamber, at least one (I) side liquid feed port that opens into the internal cylindrical chamber, and at least one tangential pressurized gas feed port that opens into the internal cylindrical chamber;
  - wherein the closed end and the open end are perpendicular to the axis of symmetry;
  - wherein the at least one (P) side liquid feed port and the at least one (I) side liquid feed port are arranged along a circumference of the internal cylindrical chamber proximate the closed end;
  - wherein the at least one tangential pressurized gas feed port is arranged along the circumference of the internal cylindrical chamber downstream of the at least one (P) side liquid feed port and the at least one (I) side liquid feed port from the closed end;
  - wherein the poly side (P) liquid component is introduced into the internal cylindrical chamber through the at

## 19

least one (P) side liquid feed port at a (P) side charge pressure of 6,895 to 27,600 kPa; wherein the iso side (I) liquid component is introduced into the internal cylindrical chamber through the at least one (I) side liquid feed port at an (I) side charge pressure of 6,895 to 27,600 kPa; wherein a combined mass flow rate of the poly side (P) liquid component and the iso side (I) liquid component to the internal cylindrical chamber is 1 to 500 g/s, wherein the poly side (P) liquid component, the iso side (I) liquid component and the pressurized gas are intermixed within the internal cylindrical chamber to form a combination; wherein the pressurized gas is introduced into the internal cylindrical chamber through the at least one tangential pressurized gas feed port with a supply pressure of 150 to 1,500 kPa; wherein an inlet velocity into the internal cylindrical chamber of the pressurized gas is 50 to 600 m/s calculated based on ideal gas conditions at 20° C. and 1 atm pressure; wherein the poly side (P) liquid component comprises 25 to 95 wt % of a (P) side polyol; wherein the (P) side polyol is a high molecular weight polyether polyol; and wherein the high molecular weight polyether polyol has a number average molecular weight, MN, of 2,500 to 100,000 and an average of 4 to 8 hydroxyl groups per molecule; discharging the combination from the open end of the internal cylindrical chamber toward the base at a velocity of 5 to 1,000 msec;

## 20

allowing the combination to solidify into a cake; separating the cake from the mold; and, deriving the chemical mechanical polishing pad polishing layer from the cake, wherein the chemical mechanical polishing pad polishing layer has a polishing surface with the groove pattern formed into the polishing surface, and wherein the polishing surface is adapted for polishing a substrate. 2. The method of claim 1, wherein the iso side (I) liquid component comprises a polyfunctional isocyanate having an average of two reactive isocyanate groups per molecule. 3. The method of claim 1, wherein the pressurized gas is selected from the group consisting of: CO<sub>2</sub>, N<sub>2</sub>, air and argon. 4. The method of claim 3, wherein the pressurized gas has a water content of ≤10 ppm. 5. The method of claim 1, wherein the internal cylindrical chamber has a circular cross section in a plane perpendicular to the axis of symmetry of the internal cylindrical chamber. 6. The method of claim 5, wherein the open end of the internal cylindrical chamber has a circular opening perpendicular to the axis of symmetry of the internal cylindrical chamber; and wherein the circular opening is concentric with the circular cross section. 7. The method of claim 6, wherein the circular opening has an inner diameter of 2.5 to 6 mm. 8. The method of claim 6, wherein the circular opening has an inner diameter of 3 mm. 9. The method of claim 1, wherein the polishing surface is adapted for polishing a semiconductor wafer.

\* \* \* \* \*